

## UNITED STATES PATENT OFFICE

2,011,176

## ORE CONCENTRATION

Cornelius H. Keller, San Francisco, Calif., assignor to Minerals Separation North American Corporation, New York, N. Y., a corporation of Maryland

No Drawing. Application March 1, 1930,  
Serial No. 432,563

8 Claims. (Cl. 209—166)

This invention relates to ore concentration with compounds of organic substituted mono-thio-carbonic acid, and is herein illustrated in froth-flotation procedures carried out with compounds containing the hydrocarbon radicals which form alcohols, such as the ethyl or benzyl alcohols. Such compounds are unsaponifiable compounds of the type



10

wherein R is a hydrocarbon radical and M is hydrogen or a metal or another



15

A number of these compounds are easily prepared in a form pure enough for ore concentration, when carbon-oxy-sulphide is passed into a solution of a caustic alkali, such as an alkali metal hydroxide, for example, potassium hydroxide, in the alcohol containing the hydrocarbon radical R selected.

These compounds are relatively cheap substances, and as illustrated below, are effective on a variety of ores when used in small amounts. It is found, for example, that iron-bearing copper ores can be concentrated by the aid of these derivatives so as to yield concentrates rich in copper and yet reject a large proportion of the undesired iron.

It may be noted that carbon-oxy-sulphide is readily and cheaply made by conducting carbon monoxide and sulphur vapor through hot clay or porcelain tubes, or subjecting such a mixture to electrical discharges. For testing purposes it has been prepared by the action of sulphuric acid on potassium sulphocyanide, being purified by passing through strong caustic soda solution and sulphuric acid.

*Example I.*—Utah copper ore was reground wet to pass 80-mesh with lime, equal to four pounds of calcium oxide per ton of dry ore, and made into a pulp with more water in a minerals separation subaeration testing machine and agitated for two minutes with 0.25 pound of potassium ethyl mono-thio-carbonate and 0.1 pound of pine oil, both per ton of ore. Froth was then removed for five minutes during continued agitation, yielding a copper concentrate. The results are shown in the following table:

| Per cent wt. | Cu analysis | Per cent Cu recovered |
|--------------|-------------|-----------------------|
| Heads 100.00 | 0.999       | 100.00                |
| Conc. 5.33   | 16.24       | 86.69                 |
| Tail. 94.67  | 0.14        | 13.31                 |

Somewhat inferior but useful results were obtained when the pulp was neutral or acid.

*Example II.*—Another lot of the same ore was similarly ground with lime and similarly agitated with 0.25 pound of potassium amyl mono-thio-carbonate and 0.1 pound of pine oil, both per ton of ore. After two minutes agitation, froth was removed for five minutes during continued agitation, yielding a copper concentrate. The results are shown in the following table:

| Per cent wt. | Cu analysis | Per cent Cu recovered | 10. |
|--------------|-------------|-----------------------|-----|
| Heads 100.00 | 1.013       | 100.00                | 15  |
| Conc. 7.73   | 11.44       | 87.27                 |     |
| Tail. 92.27  | 0.14        | 12.73                 |     |

Somewhat inferior but useful results were obtained when the pulp was neutral or acid.

*Example III.*—Another lot of the same ore was similarly ground with lime and similarly agitated with 0.1 pound of potassium ethyl mono-thio-carbonate and 0.2 pound of cresylic acid, both per ton of ore. After two minutes agitation a rougher froth concentrate was removed for five minutes during agitation. This rougher concentrate was put back into the machine with the further addition of 0.05 pound of the cresylic acid per ton of the ore, and reagitated for two minutes, and then a cleaned froth concentrate removed during three minutes agitation. The tails from this operation constituted a middling. The results are shown in the following table:

| Per cent wt. | Assays     |            |        | Recoveries |            | 40 |
|--------------|------------|------------|--------|------------|------------|----|
|              | Percent Cu | Percent Fe | Insol. | Percent Cu | Percent Fe |    |
| Heads 100.00 | 1.012      | 2.90       |        | 100.00     | 100.00     |    |
| Conc. 2.81   | 27.68      | 27.2       | 6.5    | 76.88      | 20.37      |    |
| Midd. 3.82   | 3.20       | 14.3       |        | 12.05      | 18.85      |    |
| Tail. 93.37  | 0.12       | 1.7        |        | 11.07      | 54.78      | 45 |

The large rejection of iron will be noted.

*Example IV.*—Another lot of the same ore was similarly ground with lime and similarly agitated with 0.1 pound of potassium amyl mono-thio-carbonate and 0.2 pound of cresylic acid, both per ton of ore, agitated for two minutes, and a rougher froth concentrate removed during continued agitation for five minutes. The rougher concentrate was put back into the machine and reagitated and a cleaned froth concentrate removed for three minutes. The tails from this

operation constituted a middling. The results are shown in the following table:

| 5  | Per cent wt. | Assays     |            |        | Recoveries |            |
|----|--------------|------------|------------|--------|------------|------------|
|    |              | Percent Cu | Percent Fe | Insol. | Percent Cu | Percent Fe |
| 10 | Heads 100.0  | 1.048      | 2.96       |        | 100.00     | 100.00     |
|    | Conc. 4.3    | 19.76      | 30.8       | 9.4    | 81.11      | 44.71      |
|    | Midd. 3.3    | 2.36       | 7.6        |        | 7.44       | 8.48       |
|    | Tail. 92.4   | 0.13       | 1.5        |        | 11.45      | 46.81      |

15 *Example V.*—Phelps-Dodge ore was reground wet to pass 85-mesh with lime equal to two pounds of calcium oxide per ton of dry ore, and made into a pulp with more water in a similar machine and agitated for two minutes with 0.15 pound of potassium ethyl mono-thio-carbonate, and 0.15 pound of dark cresylic acid (95-100% pure), and a rougher froth concentrate separated for ten minutes. This concentrate was reground for five minutes with one pound of calcium oxide per ton of the ore, and then reagitated with the further addition of 0.05 pound of the cresylic acid 20 per ton of the ore, and separated into a finished concentrate and a middling. The results are shown in the following table:

| 30 | Per cent wt. | Assays     |            |        | Recoveries |            |
|----|--------------|------------|------------|--------|------------|------------|
|    |              | Percent Cu | Percent Fe | Insol. | Percent Cu | Percent Fe |
| 35 | Heads 100.00 | 1.073      | 2.34       |        | 100.00     | 100.00     |
|    | Conc. 3.89   | 23.6       | 23.4       | 11.4   | 85.55      | 38.90      |
|    | Midd. 10.37  | 1.0        | 11.3       |        | 9.69       | 50.11      |
|    | Tail. 85.74  | 0.06       | 0.3        |        | 4.75       | 10.99      |

40 Results obtained with the butyl and benzyl, and with the cyclohexyl, compounds of mono-thio-carbonic acid were almost as useful as those obtained with the ethyl and amyl compounds.

45 The lead and copper salts of ethyl mono-thio-carbonic acid were also useful, especially in pulps made alkaline with lime.

50 Potassium ethyl mono-thio-carbonate also proved useful in the concentration of lead and zinc ores.

55 *Example VI.*—Ten-mesh ore of Desloge Lead Company was reground to pass 100-mesh and agitated in a pulp for five minutes with 0.2 pound of potassium ethyl mono-thio-carbonate and 0.1 pound of pine oil, both per ton of ore, and then a froth concentrate was separated for five minutes. The results are shown in the following table:

| 60          | Per cent wt. | Assay per cent Pb | Per cent recoveries |             |
|-------------|--------------|-------------------|---------------------|-------------|
|             |              |                   | Per cent Pb         | Per cent Zn |
| Heads 100.0 |              | 4.75              | 100.00              |             |
| Conc. 9.1   |              | 51.2              | 98.08               |             |
| Tail. 90.9  |              | 0.1               | 1.92                |             |

65 *Example VII.*—Ten-mesh ore from Universal Exploration Company was reground wet with two pounds of calcium oxide and one and one-half pounds of copper sulphate, both per ton of ore, until only 2% of the ore was coarser than 48-mesh and 48% passed 200-mesh. The ore was then made into a pulp with more water and agitated for five minutes with 0.3 pound of potassium ethyl mono-thio-carbonate, 0.4 pound of Barrett No. 4, and 0.15 pound of pine oil, all per ton of ore, and a rougher froth concentrate

70 separated for five minutes. This concentrate was then put back in the machine and reagitated with further addition of 0.05 pound of potassium ethyl mono-thio-carbonate per ton of original ore, agitated for two minutes, and thus was separated into a finished concentrate and a middling. The results are shown in the following table:

| Per cent wt. | Assay per cent Zn | Per cent recovery Zn |
|--------------|-------------------|----------------------|
| Heads 100.00 | 18.81             | 100.00               |
| Conc. 29.81  | 61.0              | 96.66                |
| Midd. 5.74   | 7.6               | 2.32                 |
| Tail. 64.45  | 0.3               | 1.02                 |

20 *Example VIII.*—Ten-mesh ore of the Leadville Lead-Zinc Company was reground with 6 pounds of sodium carbonate, 0.2 pound of sodium cyanide, and 2 pounds of zinc sulphate, all per ton of ore, until 94% passed 200-mesh. The ore was made into a pulp with more water and agitated for five minutes while separating a froth, with the further addition of 4 pounds of sodium carbonate, 0.1 pound of potassium ethyl mono-thio-carbonate and 0.15 pound of dark cresylic acid (95 to 100 per cent) all per ton of ore. This yielded a rougher lead concentrate, and a tailing to be treated for the recovery of the zinc. The rougher lead concentrate was put back in the machine and reagitated for ten minutes while separating a finished lead froth concentrate, there having been added 0.2 pound of potassium ethyl mono-thio-carbonate, 0.1 pound of the cresylic acid, 0.1 pound of pine oil and 0.1 pound of Barrett No. 4, all per ton of original ore. The tailing from this operation constituted a lead middling. The first tailing was agitated for ten minutes while a zinc rougher froth was separated, there having been added 5 pounds of calcium oxide, 2.5 pounds copper sulphate, 0.2 pound of potassium ethyl mono-thio-carbonate, 0.3 pound of Barrett No. 634, and 0.05 pound of pine oil, all per ton of original ore. The tailings from this operation constituted the final tailings. This rougher zinc concentrate was put back into the machine and reagitated and separated into a finished zinc concentrate and a zinc middling. The results are shown in the following table:

| 50             | Per cent wt. | Assays      |             | Per cent recoveries |        |
|----------------|--------------|-------------|-------------|---------------------|--------|
|                |              | Per cent Pb | Per cent Zn | Pb                  | Zn     |
| Heads 100.00   |              | 5.03        | 18.88       | 100.00              | 100.00 |
| Pb Conc. 2.68  |              | 74.0        | 6.0         | 39.43               | 0.85   |
| Pb Midd. 5.76  |              | 31.6        | 15.6        | 36.19               | 4.76   |
| Zn Conc. 30.69 |              | 1.2         | 54.4        | 7.32                | 88.45  |
| Zn Midd. 3.77  |              | 6.1         | 22.2        | 4.57                | 4.43   |
| Tail. 57.10    |              | 1.1         | 0.5         | 12.49               | 1.51   |

65 *Example IX.*—Ten-mesh Parroquia ore from Zacatecas, Mexico, was reground in a laboratory ball mill with water with 6 pounds sodium carbonate, 0.2 pound sodium cyanide, and 3 pounds of zinc sulphate, all per ton of ore, until 91.5% passed 200 mesh. The ore was made into a pulp with water and agitated for 7 minutes during the separation of a rougher copper-bearing froth, there having been added 0.15 pound per ton of potassium ethyl mono-thio-carbonate and 0.2 pound of the cresylic acid, both per ton of ore. The tailings from this operation were later used for the recovery of zinc. This rougher froth concentrate was put back into the machine and re-

5 agitated for three minutes during froth separation, there having been added 1 pound of zinc sulphate and 0.1 pound of the cresylic acid, both per ton of ore, and separated into a finished copper concentrate and a copper middling. The first tailing was then put back into the machine with the further addition of one pound of copper sulphate, 0.15 pound potassium ethyl-mono-thiocarbonate and 0.3 pound of Barrett No. 634, all 10 per ton of ore, and agitated with froth separation for seven minutes to yield a rougher zinc froth concentrate. The tailings from this operation constituted the final tailings. The rougher zinc froth concentrate was then put back into the machine and agitated for five minutes with the separation of a finished zinc froth concentrate, there having been added 0.1 pound of potassium ethyl-mono-thio-carbonate, 0.05 pound Barrett No. 634, and 0.05 pound pine oil, all per 15 ton of ore. The tailings from this operation constituted a zinc middling. The results are shown in the following table:

| 25             | Per cent wt. | Assays     |            |            | Recoveries |            |
|----------------|--------------|------------|------------|------------|------------|------------|
|                |              | Percent Pb | Percent Cu | Percent Zn | Percent Cu | Percent Zn |
| 30             | Heads 100.00 | 1.38       | 16.60      | 100.0      | 100.00     |            |
| Cu Conc. 2.19  | 10.8         | 21.04      | 12.8       | 33.3       | 1.69       |            |
| Cu Midd. 3.19  | 6.0          | 6.0        | 26.08      | 13.8       | 5.15       |            |
| Zn Conc. 30.31 | 2.0          | 45.0       | 43.8       | 82.17      |            |            |
| Zn Midd. 4.79  | 1.16         | 23.2       | 4.0        | 6.69       |            |            |
| Tail. 59.52    | 0.12         | 1.2        | 5.1        | 4.30       |            |            |

35 *Example X.*—Ten-mesh ore from Mazapil Copper Company, representing material from No. 2 waste dump and largely oxidized, was reground wet until 90% passed 200-mesh. The ground material was made into a pulp with water and agitated for five minutes with 0.1 pound of potassium ethyl-mono-thio-carbonate and a first froth concentrate separated. The remaining pulp was then further agitated for five minutes with 2 pounds sodium sulphide, 2 pounds potassium ethyl mono-thio-carbonate, 0.25 pound Barrett No. 4, and 0.1 pound pine oil, all per ton of ore. A froth concentrate was then separated for five minutes, and a large part of the oxidized copper mineral was recovered in the concentrate. The results are shown in the following table:

|             | Per cent wt. | Per cent Cu assay | Per cent Cu recovery |
|-------------|--------------|-------------------|----------------------|
| 55          | Heads 100.0  | 2.175             | 100.00               |
| Conc. 1 3.9 | 29.76        | 53.28             |                      |
| Conc. 2 6.6 | 9.40         | 28.51             |                      |
| Tail. 89.5  | 0.44         | 18.21             |                      |

60 *Example XI.*—Ten-mesh Colossus Mining Company ore was reground wet until 74% passed 200 mesh. The ground ore was made into a pulp with water and agitated with 0.3 pound of potassium ethyl mono-thio-carbonate, 0.6 pound of Barrett No. 4, 0.15 pound pine oil, all per ton of ore, and a rougher froth concentrate separated for seven minutes during the agitation. The concentrate thus obtained was put back in the machine and reagitated with 0.05 pound of the potassium ethyl mono-thio-carbonate and 0.05 pound of pine oil, both per ton of original ore, and a finished froth concentrate separated, the tailings from this operation constituting a middling. The recovery of values was about the same as in the best results hitherto obtained, and the ratio 65 of concentration was superior to any obtained

with concomitant large recoveries. The results are shown in the following table:

| Per cent Wt. | Assays |        | Recoveries  |             |
|--------------|--------|--------|-------------|-------------|
|              | Oz. Au | Oz. Ag | Per cent Au | Per cent Ag |
| Heads 100.00 | 0.61   | 30.94  | 100.00      | 100.00      |
| Conc. 1.91   | 30.18  | 1466.0 | 94.23       | 90.49       |
| Midd. 5.61   | 0.30   | 29.4   | 2.75        | 5.33        |
| Tail. 92.48  | 0.02   | 1.4    | 3.02        | 4.18        |

15 In addition to the salts of ethyl mono-thiocarbonic acid other compounds may be used such as the disulphide obtained when potassium ethyl mono-thio-carbonate is treated with ferricyanide of potassium, such disulphide being variously designated as ethyl-carbonic acid disulphide and dicarbethoxy disulphide.

20 *Example XII.*—Utah Copper Company ore was wet ground for ten minutes so that the ore passed 80-mesh and was then made into a pulp with water and agitated with 0.1 pound of pine oil and 0.25 pound of the disulphide described above, both per ton of ore, to yield a froth concentrate of 11.60% copper and tailings of 0.28% copper, representing a recovery of 75.5% of the copper.

25 *Example XIII.*—Another similar lot of the same ore similarly ground was made into a pulp and agitated with the pine oil and the disulphide aforesaid and with the further addition of 7 pounds of sulphuric acid per ton of ore, to yield a froth concentrate. This lot of ore contained 1.058% copper, the concentrate 11.28% copper, and the tailings 0.12% copper, representing a recovery of 89.6% of the copper.

30 *Example XIV.*—Another similar lot of the same ore was ground similarly but with the addition of lime equal to 4 pounds per ton of the ore, and then made into a pulp and agitated with the pine oil and the disulphide aforesaid, to yield a froth concentrate. This lot of the ore contained 0.966% of copper, the concentrate 12.56% copper, and the tailings 0.13% copper, representing a recovery of 87.47% of the copper.

35 Having thus described certain embodiments of the invention, what is claimed is:

40 1. The process of concentrating an ore carrying gangue and a value which consists in agitating and aerating a pulp of the ore with a mineral-frothing agent and a compound of the type



45 in an amount of less than half a pound per ton of the ore, wherein R is a hydrocarbon radical and M is a hydrogen or a metal or another



50 so as to obtain a floating concentrate substantially dependent upon the presence of the compound for an enhanced proportion of value and diminished proportion of gangue in the concentrate compared with a concentrate obtained in the absence of the compound.

55 2. The process of concentrating an ore carrying gangue and a value which consists in agitating and aerating a pulp of the ore with a mineral-frothing agent and a compound containing an alkyl substituted mono-thio-carbonic acid radical in an amount of less than half a pound per ton of the ore so as to obtain a floating concentrate substantially dependent upon the presence of the

55

60

65

70

75

- compound for an enhanced proportion of value and diminished proportion of gangue in the concentrate compared with a concentrate obtained in the absence of the compound.
5. 3. The process concentrating an ore carrying gangue and a value which consists in agitating and aerating a pulp of the ore with a mineral-frothing agent and with a salt of an alkyl substituted mono-thio-carbonic acid in an amount 10 of less than half a pound per ton of the ore so as to obtain a floating concentrate substantially dependent upon the presence of the salt for an enhanced proportion of value and diminished proportion of gangue in the concentrate compared 15 with a concentrate obtained in the absence of the salt.
4. The process of concentrating an ore carrying gangue and a value which consists in agitating and aerating a pulp of the ore with a mineral-frothing agent and an ethyl mono-thio-carbonate in an amount of less than half a pound per ton of the ore so as to obtain a floating concentrate substantially dependent upon the presence of the carbonate for an enhanced proportion 20 of value and diminished proportion of gangue in the concentrate compared with a concentrate obtained in the absence of the carbonate.
5. The process of concentrating an ore carrying gangue and a value which consists in agitating and aerating a pulp of the ore with a mineral frothing agent and a salt of ethyl-mono-thio-carbonic acid in an amount of less than half a pound per ton of the ore so as to obtain a floating concentrate substantially dependent upon the presence of the salt for an enhanced proportion of value and a diminished proportion of gangue in the concentrate compared with a concentrate obtained 25 in the absence of the salt.
6. The process of concentrating an ore carrying gangue and a value which consists in agitating and aerating a pulp of the ore with a mineral-frothing agent and an alkali salt of ethyl mono-thio-carbonic acid in an amount of less than half a pound per ton of the ore so as to obtain a floating concentrate substantially dependent upon the presence of the salt for an enhanced proportion of value and a diminished proportion of gangue in the concentrate compared with a concentrate obtained in the absence of the salt. 5
7. The process of concentrating a copper ore carrying gangue and a normally floatable iron mineral which consists in agitating and aerating a pulp of the ore with a mineral-frothing agent and with a salt of an alkyl-substituted mono-thio-carbonic acid in an amount of less than half a pound per ton of the ore so as to obtain a floating concentrate substantially dependent upon the presence of the salt for an enhanced proportion of copper and a diminished proportion of gangue and of iron in the concentrate compared with a concentrate obtained in the absence of the salt. 15
8. The process of concentrating a copper ore carrying gangue and a normally floatable iron mineral which consists in grinding the ore with lime, agitating and aerating a pulp of the ground ore with a mineral-frothing agent and a salt of ethyl substituted mono-thio-carbonic acid so as to obtain a floating concentrate substantially dependent upon the presence of the salt for an enhanced proportion of copper and a diminished proportion of gangue and of iron in the concentrate compared with a concentrate obtained 20 in the absence of the salt. 25
- 30
- 35

CORNELIUS H. KELLER.